

## 1

3,510,321

### SEALANT FOR PIPE JOINTS

Robert L. Turner, 2127 N. Keebler Road,  
Collinsville, Ill. 62234

No Drawing. Filed Dec. 23, 1968, Ser. No. 786,401  
Int. Cl. G09k 3/10

U.S. Cl. 106—33

5 Claims

### ABSTRACT OF THE DISCLOSURE

A sealing compound for pipe joints and the like consisting principally of ferric oxide and glycerine, preferably in the proportion of five parts of ferric oxide powder and two parts of glycerine is nonhardening so that pipes sealed with it can be separated without danger of stripping the threads and the compound, as distinguished from some prior art sealants, can be used in pipes through which oxygen passes.

### BACKGROUND OF THE INVENTION

#### Field of the invention

The invention relates to a sealing compound for threaded pipe joints and the like which provides a non-hardening seal which is not subject to deterioration from oxygen.

#### Description of the prior art

The most common sealant for pipe joints has been glycerine litharge cement consisting of a mixture of glycerine and lead oxide. Although glycerine litharge cement provides an effective seal for pipe joints, it has the serious disadvantage that it becomes extremely hard as it ages. Hence it cannot be prepared in advance of use and stored and it is difficult to disassemble pipe joints sealed with it without stripping their threads.

### SUMMARY OF THE INVENTION

The invention provides a nonhardening oxygen-resistant threaded pipe joint sealing compound which has these properties by virtue of the principal ingredients of the compound, namely, ferric oxide and glycerine.

### DESCRIPTION OF THE PREFERRED EMBODIMENT

The ingredients of my sealing compound and the proportions thereof are as follows:

|                     | Parts  |
|---------------------|--------|
| Ferric oxide powder | 4 to 7 |
| Glycerine           | 2      |

I have found that most satisfactory results can be obtained with 5 parts of ferric oxide powder to 2 parts of glycerine.

## 2

The compound is prepared by thoroughly mixing the ferric oxide powder and glycerine together to a consistency similar to that of thick paint. It can be stored indefinitely in sealed containers; it is applied to pipe joints by coating the threads before joining them.

The ferric oxide powder which I have used successfully in this compound is a waste product of steel plants consisting of the following ingredients in the percentages shown:

|              | Percent |
|--------------|---------|
| Ferric oxide | 97.3    |
| Silica       | 2.2     |
| Graphite     | 0.1     |
| Calcium      | Trace   |

15 The silica, graphite and calcium are impurities present in the powder, and with the possible exception of the graphite, are believed to contribute nothing to the efficacy of the compound.

20 The compound is harmless to use, inexpensive to make, provides a stable oxygen-resistant seal and, unlike glycerine litharge cement, it will not set up or harden irrespective of how long the joint remains in service, so that if it becomes necessary to disassemble the joint, the joint members can be freely unscrewed without damage to the threads. It is believed that the presence of graphite may be reason of its lubricating properties enhance the ease of assembling and disassembling joints coated with the compound.

25 I claim:

- 30 1. A compound for sealing pipe joints and the like consisting by volume of substantially four to seven parts of ferric oxide powder and two parts of glycerine.
2. A compound according to claim 1 containing by volume substantially four parts of ferric oxide powder and two parts of glycerine.
- 35 3. A compound according to claim 1 containing by volume substantially five parts of ferric oxide powder and two parts of glycerine.
4. A compound according to claim 1 containing by volume six parts of ferric oxide powder and two parts of glycerine.
5. A compound according to claim 1 containing by volume seven parts of ferric oxide powder and two parts of glycerine.

### References Cited

#### UNITED STATES PATENTS

604,532 5/1898 Jewett ----- 106—3

50 JULIUS FROME, Primary Examiner

T. MORRIS, Assistant Examiner

U.S. Cl. X.R.

106—287